

## UNITED STATES PATENT OFFICE.

WILLIAM A. L. SCHAEFER, OF CHICAGO, ILLINOIS, ASSIGNOR TO PLIBRICO JOINTLESS FIREBRICK COMPANY, OF CHICAGO, ILLINOIS, A CORPORATION OF ILLINOIS.

## PLASTIC FIRE BRICK.

No Drawing.

Application filed April 9, 1919. Serial No. 288,745.

*To all whom it may concern:*

Be it known that I, WILLIAM A. L. SCHAEFER, a citizen of the United States, residing at Chicago, in the county of Cook and State of Illinois, have invented a certain new and useful Improvement in Plastic Fire Brick, of which the following is a full, clear, concise, and exact description.

My invention relates to plastic fire brick 10 and method of making same and contemplates a new plastic fire brick, as a composition of matter, and a new process by means of which this new composition of matter is prepared.

As is well known in the art, so called plastic fire brick is used for the building of one piece furnace linings, arches and bridge walls set in largely the same manner that concrete structures are set, and the objects 20 of my invention are:

(a) To provide an efficient, plastic fire brick of abundantly available materials;

(b) To provide an efficient plastic fire brick which will not deteriorate between its 25 original preparation and its use;

(c) To provide an efficient, plastic fire brick which can readily be prepared for installing.

(d) To provide an efficient, plastic fire brick which will hold together in large 30 masses and which will be durable when installed and baked;

(e) To provide a plastic fire brick of suitably high fusing point; and

(f) To provide a process whereby this fire 35 brick can be produced economically.

To the ends above noted, I have, by extended experimentation, determined a certain composition of matter, which I have 40 proven out by test and actual use, and which I shall set forth and claim hereinafter.

With reference first to the clay which I employ, assuming silica, of course, to be the main ingredient, I select a clay as high as 45 possible in alumina, and as low as possible in sodium oxide, potassium oxide, lime, magnesia, iron oxide and titanium oxide. To this end I employ a clay, abundant in quantity available, as follows:

Silica, from 50 to 62 per cent; alumina, 50 from 30 to 40 per cent; iron and titanium oxide, from 1.5 to 3 per cent; lime, from .1 to 1.5 per cent; alkalies, from .1 to 1.5 per cent; magnesia, from .05 to .35 per cent; with sodium and potassium oxides only in trace, apportioned into raw and calcined parts in the proportion of nine and two and mixed together and with ground burned fire-brick in the proportion of eleven and eighteen.

with sodium and potassium oxides only in 55 trace.

Of clay of this type I employ two portions, in the proportion of approximately nine parts and two parts, and the smaller portion of which is calcined. I thereupon 60 mix these two portions and then add to them, considering them as eleven parts, approximately eighteen parts of ordinary burned (such as used) fire brick ground and passed through a quarter inch mesh 65 screen. This entire mass is then mixed thoroughly dry, preferably by the use of suitable agitators, and, later, in the course of which mixing sufficient water to effect a stiff plastic condition is added. The material is then ready for storage for use, and when used is brought back to its original plastic condition by the addition of water if it has become too dry.

Where I employ the terms rich in alumina 75 and low in iron, I intend that the quantitative values represented by these terms be generally as set out in the analysis hereinbefore given.

The plastic fire brick, thus compounded 80 and processed, fuses at approximately three thousand degrees Fahrenheit, and is otherwise of the characteristics set forth as desirable ones at the outset of this specification.

I claim:

1. A plastic fire-brick comprising a clay rich in alumina apportioned into raw and calcined parts in the proportion of nine and two mixed together and with ground burned 90 fire-brick in the proportion of eleven and eighteen.

2. A plastic fire-brick comprising a clay of the following characteristics: Silica, from 50 to 62 per cent; alumina, from 30 to 40 per cent; iron and titanium oxide, from 1.5 to 3 per cent; lime, from .1 to 1.5 per cent; alkalies, from .1 to 1.5 per cent; magnesia, from .05 to .35 per cent; with sodium and potassium oxides only in trace, apportioned into raw and calcined parts in the proportion of nine and two and mixed together and with ground burned fire-brick in the proportion of eleven and eighteen.

In witness whereof, I hereunto subscribe 105 my name, this 24th day of March, 1919.

WILLIAM A. L. SCHAEFER.